

## UNITED STATES PATENT OFFICE

2,330,163

## PROCESS FOR THE SIMULTANEOUS PRODUCTION OF PETROLEUM SULPHONIC ACID BODIES AND A STABLE LUBRICATING OIL

Pharez G. Waldo, Paul M. Goodloe, 2nd, and Henry G. Berger, Woodbury, N. J., assignors to Socony-Vacuum Oil Company, Incorporated, New York, N. Y., a corporation of New York

No Drawing. Application March 8, 1940,  
Serial No. 322,970

## 5 Claims. (Cl. 196—40)

This invention relates to the treatment of petroleum solvent tars. More particularly the invention relates to the production of stable lubricating oils from petroleum solvent tars.

It is an object of our invention to provide useful products from petroleum solvent tars.

A more specific object of our invention is to provide a method of obtaining stable lubricating oils from solvent tars.

Still another object is to provide a practical use for petroleum solvent tars.

A further object is to provide useful sulphonated solvent tar products.

For many years lubricating oil fractions were acid treated with sulphuric acid to remove undesirable constituents such as unsaturates, etc. With the advent of solvent refining, acid treating of lubricating oils was greatly reduced, since, as is well known, the solvents preferentially extracted the undesirable constituents leaving the desirable constituents. Many solvents have been proposed and used in the solvent refining of petroleum oils, as for instance, furfural, sulphur dioxide, Chlorex (dichloro-diethyl ether) etc. Also combinations of solvents such as acetone and benzol have been used. Still further a precipitant for undesirable constituents, such as propane, and a solvent, such as cresylic acid, have been used together. Propane has also been used alone as an asphalt precipitant, in order to precipitate a substantially oil-free asphaltic product, however, this invention is not concerned with such a product. In the usual solvent refining processes, a raffinate and an extract or solvent tar are produced. The raffinate is the refined oil. The extract or solvent tar contains undesirable constituents extracted by at least one solvent therefor.

Heretofore solvent tars have been thought of generally as products containing only undesirable constituents insofar as lubricants are concerned. Accordingly, while portions of solvent tars have been used as fuel oils and for other uses, it is quite surprising to find that a stable lubricating oil may be produced from solvent tars.

According to our invention a petroleum solvent tar which has been extracted from a lubricating oil distillate fraction by solvent refining, is subjected to a relatively heavy acid treatment sufficient to sulphonate a portion thereof to yield a sulphonated solvent tar product and an unsulphonatable oil, the unsulphonatable oil is then further refined or treated to produce a finished lubricating oil which is stable to

oxidation. The solvent tars or extracts used in our invention must, of course, be derived from the treatment of sufficiently heavy fractions to contain hydrocarbons of lubricating oil range.

As has been indicated above, there are numerous petroleum solvent tars or extracts produced by the use of numerous solvents and combinations thereof, e. g., furfural, liquid sulphur dioxide, Chlorex, benzol-acetone, Duo-Sol (propane and cresylic acid) etc. Moreover, these solvent tars are produced from nearly every type of crude, comprising in each case the less paraffinic portions of the oil treated. In accordance with our invention any of these solvent tars or extracts from a distillate oil may be used to obtain our stable lubricating oil, and we particularly prefer furfural and Chlorex tars.

The solvent tar sulphonic acids produced by our process may be recovered by any of the well known procedures for recovering sulphonic acids from mineral oils in general. After removal of the sulphonic acids or sulphonates there remains a mineral oil which is essentially unsulphonatable and which, after blowing bright, to remove occluded water, etc., represents usually from about 10% to 60% of the original solvent tar.

The unsulphonatable oil remaining after the sulphonates are extracted, will require some further treating or refining in order to make a finished lubricant. This required treating will depend somewhat on the previous history and nature of the oil. Usually the oil must be blown bright, as noted above, to remove occluded matter and give a bright appearance. Further, de-waxing may be necessary followed by treatment with clay to give proper color.

The sulphonation of mineral oil fractions in general is well known as likewise is the recovery of the sulphonated products. However, in order to further illustrate the present invention wherein solvent tars are sulphonated, the following specific examples are given:

## EXAMPLE I

45 A furfural extract of A. P. I. gravity of 12.8 and S. U. V. at 210° F. of 39 which was obtained in 27.5% yield by treating a Mirando distillate (Coastal) of A. P. I. gravity of 20.2 and S. U. V. at 210° F. of 38.5 with 150% by volume of furfural at 130 to 200° F. was treated with 10% by volume of 94% sulphuric acid, 10% by volume of 98% acid, and then 3 times with 10% by volume of oleum each time, separating the sludge between each dump. The total amount of oleum used was 115 lbs. per bbl. of tar. The

yield of sulphonates was 11.8% by weight of the starting furfural tar, obtained by extracting the sulphonated oil with dilute alcohol after each oleum dump. The sulphonated material obtained from this furfural tar has the novel property that the free sulphonic acids are soluble in oil, whereas their sodium salts are insoluble in the same oil. These sodium sulphonates may be used as detergents.

#### EXAMPLE II

A furfural extract of A. P. I. gravity of 19.1 and S. U. V. at 210° F. of 51 was obtained as a 34% yield by treating a Wewoka distillate (Mid-Continent) of A. P. I. gravity of 28.4 and S. U. V. at 210° F. of 44 with 250% by volume of furfural at 200 to 260° F. This extract was treated with 60 lbs. per barrel of 98% sulphuric acid to remove sludge forming materials. The extract was then diluted with an equal volume of recovered oil from a former treatment of the same tar, and sulphonated with 200 lbs. of oleum per barrel in three equal dumps, separating the sludge between each dump. The yield of sulphonates obtained on extracting the acid oil, freeing the extract of mineral oil by washing with naphtha, neutralizing with strong caustic soda, filtering and evaporating, amounted to 16.1% by weight of the starting furfural tar.

The sulphonates from the above Wewoka furfural tar were light colored and quite soluble in a petroleum oil of A. P. I. gravity of 29.0 to 29.2 and S. U. V. at 100° F. of 100 to 110 seconds. The sulphonates were stable to light, possessed excellent emulsifying activity and were non-corrosive to iron. About 10% by weight, or less, with about 10% rosin soap in oil gave a good soluble cutting oil which formed stable 1 to 15 emulsions in soft water and in hard water containing 1000 parts per million hardness.

The oil left after extracting the sulphonates from the sulphonated Wewoka tar was blown bright, dewaxed at -20° F. with toluol-acetone and percolated through 10% of its weight of fresh burnt 30-60 fuller's earth at 120-130° F.

The following tests were obtained on this oil; a blend (A-W) of 25% of this oil with 75% of a standard turbine oil (A); and on the standard turbine oil (A).

10

|                        |                       | Wewoka oil | Blend A-W | Standard A <sup>1</sup> |
|------------------------|-----------------------|------------|-----------|-------------------------|
| 15                     | A. P. I. gravity..... | degrees    | 30.1      | 29.6                    |
| Pour.....              | ° F.                  | 0          | 0         | 0                       |
| Flash.....             | ° F.                  | 400        | 405       | 380                     |
| Fire.....              | ° F.                  | 465        | 465       | 450                     |
| S. U. V. @ 100° F..... | seconds               | 164        | 155       | 152                     |
| S. U. V. @ 210° F..... | do                    | 43.4       | 42.9      | 42.6                    |
| V. I.....              |                       | 82         | 86        | 88                      |
| Color, Lovibond.....   |                       | 0.5        | 0.35      | 0.3                     |
| 20                     | S. E. N.....          | minutes    | 1/4       | 1/4                     |
| N. N.....              |                       | NH         | NH        | NH                      |
| Sludge.....            | milligrams            | 6          | 13        | 13                      |
| German tar.....        | per cent              | 0.04       | 0.08      | 0.07                    |
| Brown-Boveri:          |                       |            |           |                         |
| Color, Story.....      |                       | 3          | 26.5      | 37                      |
| Color, Lovibond.....   |                       | 2          | 19        | 26                      |
| 25                     | N. N.....             | 0.01       | 0.11      | 0.07                    |
| Sludge.....            |                       | 0          | 0         | 0                       |

<sup>1</sup> Standard A is a mixed Mid-Continent and Coastal distillate which has been acid-treated and then clayed.

<sup>2</sup> Clear—no ppt.

30 The particular type oil obtained by our process will, of course, depend upon the fraction from which the solvent tar is obtained. It will be noted that the above Wewoka oil was in the turbine oil range.

35 In a manner similar to that outlined above, oils have been prepared by our process from various solvent tars of various crude fractions. In order to further illustrate the invention, the properties of many of these oils are set forth 40 in the following tabular data:

TABLE I  
Tests on recovered oil

|                                | Sample No.         |                   |      |      |        |        |       |       |       |       |       |       |
|--------------------------------|--------------------|-------------------|------|------|--------|--------|-------|-------|-------|-------|-------|-------|
|                                | 1<br>Standard<br>A | 2<br>Blend<br>A-W | 3    | 4    | 5      | 6      | 7     | 8     | 9     | 10    | 11    | 12    |
| Yield..... per cent by vol.    |                    |                   |      |      |        |        |       |       |       |       |       |       |
| Furfural tar.....              |                    |                   | 35   | 35   | Wewoka | Wewoka | 20    | 37.3  | 40    | 55    | 55    | 17.3  |
| Dilution.....                  |                    |                   |      |      | 1:1    | 2:1    | 2:1   | 2:1   | 50    | 50    | 2:1   | 2:1   |
| Dilution.....                  |                    |                   |      |      | 60     | 60     | 60    | 60    | 50    | 50    | 50    | 60    |
| Lbs./bbl. 98-R acid.....       |                    |                   |      |      | 60     | 60     | 60    | 60    | 50    | 50    | 50    | 50    |
| Gravity..... ° A. P. I.        | 29.5               | 29.6              | 29.7 | 28.3 | 30.3   | 34.6   | 30.2  | 31.8  | 15.7  | 15.5  | 40.1  | 42.0  |
| Pour..... ° F.                 | 0                  | 0                 | 75   | 70   | 75     | 15     | 5     | 5     | -20   | -25   | 115   | 400   |
| Flash..... ° F.                | 380                | 405               | 410  | 395  | 395    | 410    | 405   | 330   | 330   | 330   | 32.5  | 30.4  |
| Fire..... ° F.                 | 450                | 465               | 470  | 460  | 465    | 470    | 465   | 375   | 375   | 375   | 10    | 15    |
| S. U. V. @ 100° F.....         | 152                | 155               | 164  | 182  | 144    | 106.2  | 161.8 | 148.8 | 174.9 | 174.9 | 134.1 | 128.4 |
| S. U. V. @ 210° F.....         | 42.6               | 42.9              | 43.6 | 44.2 | 42.7   | 40.6   | 43.7  | 43.4  | 40.1  | 40.1  | 42.0  | 41.2  |
| V. I.....                      | 77                 | 86                | 88   | 77   | 95     | 123    | 100   | 110   | -108  | -108  | 98.5  | 88    |
| Color, Lovibond.....           | 0.3                | 0.35              | 1    | 0.9  | 0.45   | <0.1   | 0.55  | 0.45  | 2.4   | 2.2   | <0.1  | 0.2   |
| S. E. N..... minutes           | 1/4                | 1/2               | 3/4  | 3.4  | 1/2    | 1/2    | 1/2   | 1     | 21/2  | 1/2   | 1/2   | 1/2   |
| N. N.....                      |                    |                   | NH   |      | NH     | 0.02   | 0.01  | 0.01  | 0.05  | 0.03  | NH    | 0.02  |
| Sludge..... milligrams         | 13                 | 13                | 9    | 13   | 9      | 8.0    | 8     | 7     | 17    | 24    | 8.4   | 13    |
| German tar..... per cent wt.   | 0.07               | 0.08              | 0.11 | 0.10 | 0.09   | 1.6    | 0.09  | 0.03  | 0.65  | 0.49  | 9.6   | 0.06  |
| Brown-Boveri turbine test:     |                    |                   |      |      |        |        |       |       |       |       |       |       |
| Color, Story.....              | 37                 | 26.5              | 14   | 49   | 8.5    | 0      | 14    | 32    | 532   | 904   | 0     | 13    |
| Color, Lovibond.....           | 26                 | 19                | 10   | 38   | 5.8    | 0      | 9     | 30    | 260   | 370   | 0     | 8     |
| N. N.....                      | 0.07               | 0.11              | 0.01 | 0.19 | 0.09   | NH     | 0.07  | 0.22  | 0.31  | 0.29  | 0.55  | 0.06  |
| Sludge..... milligrams         | 0                  | 0                 | 0    | 0    | 0      | 0      | 0     | 7     | 0     | 0     | 0     | 0     |
| S-V turbine test: <sup>1</sup> |                    |                   |      |      |        |        |       |       |       |       |       |       |
| Tube No. 1                     | 1                  | 1                 | 1    | 1    | 1      | 1      | 1     | 1     | 1     | 1     | 1     | 1     |
| Time..... days 4               | 4                  | 4                 | 4    | 4    | 4      | 4      | 4     | 4     | 4     | 4     | 4     | 4     |
| Time..... hours 90             | 90                 | 90                | 90   | 90   | 90     | 90     | 98    | 98    | 91    | 91    | 90    | 90    |
| Color, Lovibond..... 11        | 7                  | 5.8               | 11.5 | 2.4  | 0.8    | 10     | 10    | 55    | 80    | 80    | Green | 2.8   |
| N. N..... 0.57                 | 0.26               | 0.11              | 0.29 | 0.09 | 0.1    | 0.34   | NH    | 0.64  | 0.31  | 3.9   | 3.9   | 0.08  |
| Sludge..... milligrams 10      | 12                 | 1                 | 12   | 11   | 47     | 20     | 20    | 10    | 13    | 210   | 210   | 35    |
| Tube No. 2                     | 2                  | 2                 | 2    | 2    | 2      | 2      | 2     | 2     | 2     | 2     | 2     | 2     |
| Time..... days 8               | 8                  | 8                 | 8    | 7    | 8      | 8      | 8     | 8     | 8     | 7     | 7     | 8     |
| Time..... hours 186            | 186                | 186               | 186  | 186  | 162    | 186    | 191   | 191   | 185   | 185   | 164   | 186   |
| Color, Lovibond..... 60        | 53                 | 45                | 72   | 8.4  | Green  | 70     | 105   | 135   | 205   | 240   | 20    | 20    |
| N. N..... 2.4                  | 2.2                | 2.3               | 1.8  | 0.63 | 18.6   | 2.3    | 6.3   | 1.3   | 0.44  | 18.6  | 1.5   | 1.5   |
| Sludge..... milligrams 35      | 42                 | 14                | 10   | 30   | 107    | 28     | 45    | 34    | 49    | 352   | 352   | 36    |

<sup>1</sup> The S-V turbine test comprises heating 25 cc. of oil samples at 196° F. in the presence of copper, iron and water for increasing periods of time and noting the progressive changes taking place in the oil in respect to acid, color and sludge formation.

It will be noted that in general all of the above oils produced by our invention are substantially equal to, or even superior to, standard lubricating oils, particularly when the proper amount of sulphonation has been used. The oils from the highly naphthenic Mirando solvent tar, as can be noted, gave unusually good turbine oil tests; however, these particular oils do not show up quite so well under other test conditions of oxidation.

It is important that the solvent tars not be undertreated or overtreated with the sulphuric acid during sulphonation. For instance in Table I above, it may be noted that the oils of columns 6 and 11 are obviously overtreated. The proper treatment for producing the best oils will usually be found to be the proper treatment for producing sulphonates. In many cases it may be found preferable to dilute the solvent tar being treated with unsulphonated oil rather than cut down the amount of acid used. It will be noted that such procedure was followed in the specific Example II and in certain of the runs of Table I.

Since solvent tars vary considerably in the amount and nature of undesirable constituents contained therein, the amount of acid treatment must necessarily vary, however, the optimum conditions of treatment may soon be arrived at by a few adjustments, particularly since the sulphonation of petroleum fraction is so well known to the petroleum art. In general, the solvent tar usually is first treated with about 94% and/or 98% sulphuric acid to remove sludge forming materials and then with about 100 to 400 lbs. per bbl. of oleum to effect the production of sulphonic acids. As is well known in the field of sulphonic acid production, the oleum may be added in either one or several dumps, preferably in a plurality of dumps in the usual operation.

In addition to the stable oils that are produced by our process, it will be noted that mineral oil sulphonates are produced from the solvent tar as a by-product. These sulphonates may be used in the manner in which any such sulphonates are now used, depending upon whether they are oil or water soluble. For instance, the oil soluble solvent tar sulphonates may be used in soluble oils and the water soluble sulphonates may be used as detergents. We have found that, in general, when the solvent tars have an A. P. I. gravity below about 16 they produce water soluble, relatively oil insoluble sulphonates, while if the original solvent tar has an A. P. I. gravity above about 16 the resultant

sulphonates are oil soluble and relatively water insoluble.

We claim:

1. A process for the simultaneous production of petroleum sulphonic acid bodies and a stable lubricating oil which comprises subjecting solvent extract of a distillate lubricating oil stock to a sulphonation treatment with strong sulphuric acid to obtain a substantial amount of unsulphonated oil containing petroleum sulphonic acids dissolved therein, separating said sulphonic bodies remaining in the unsulphonated oil from such oil, and thereafter refining the unsulphonated oil so as to produce a stable lubricating oil therefrom.
2. The process of claim 1 wherein the sulphonation treatment of the solvent extract is carried out in the presence of added unsulphonated petroleum oil which has been obtained from the product of a sulphonation treatment of a similar oil.
3. A process for the simultaneous production of a petroleum sulphonate and a stable lubricating oil which comprises subjecting a furfural solvent extract of a distillate lubricating oil stock to a sulphonation treatment with strong sulphuric acid to obtain a substantial amount of unsulphonated oil containing petroleum sulphonic acids dissolved therein, recovering said sulphonic acids remaining in the unsulphonated oil as a sulphonate product, and thereafter refining the unsulphonated oil so as to produce a stable lubricating oil.
4. The process of claim 1 wherein the solvent extract being sulphonated has an A. P. I. gravity below about 16.
5. A process for the simultaneous production of a water soluble, substantially oil insoluble, mahogany petroleum sulphonate and a stable lubricating oil which comprises subjecting a distillate lubricating oil stock furfural solvent extract having an A. P. I. gravity below 16 to a sulphonation treatment with strong sulphuric acid to obtain a substantial amount of unsulphonated oil, containing mahogany sulphonic acids dissolved therein, recovering said sulphonic acids remaining in the unsulphonated oil as a water soluble, substantially oil insoluble sulphonate, and thereafter refining the unsulphonated oil so as to produce a stable lubricating oil.

PHAREZ G. WALDO,  
PAUL M. GOODLOE, 2ND.  
HENRY G. BERGER.